

## UNITED STATES PATENT OFFICE

HENRY PHILIP SHOPNECK, OF DORCHESTER, MASSACHUSETTS, ASSIGNOR, BY MESNE ASSIGNMENTS, TO ARDEN BOX TOE COMPANY, OF WATERTOWN, MASSACHUSETTS, A CORPORATION OF MASSACHUSETTS

## WATER-LAID FELT AND ARTICLE MADE THEREFROM

No Drawing.

Application filed January 13, 1927. Serial No. 161,025.

The problem of producing a water-laid felt, suitable for use as box toe stock for example, is complicated by the characteristics of the different fibres which may be employed 5 in the mix. Usually the felt is a wool felt containing some cotton, and the usual process of making such a felt consists in beating out the fibres in a beater in the presence of water and running them on a cylinder felt- 10 ing machine after which the stock is sheeted out and impregnated with a thermoplastic binder, usually of resinous, asphaltic or bituminous origin.

It has been proposed to make a water-laid 15 felt of beaten textile rags and to substitute fibred tannery hair for the expensive wool fibres. It has been also proposed to use in such a felt relatively long mineral or vegetable fibres in place of the tannery hair.

20 The several different kinds of fibres which are capable of being used in a beaten water-laid felt, however, have characteristically different felting actions, and the strength and stretch of the ultimate felt therefore de- 25 pends upon the particular fibre which is used.

For example, if all long fibred wool stock is used, the stock is too fluffy and will not felt on a cylinder felting machine. Nor will it 30 felt properly if all short fibred wool stock is used. If long cotton fibres are substituted for the long wool fibres in the felt made on the cylinder machine, the material cannot be kept open and porous enough to hold a sufficient amount of thermoplastic binder properly to

35 impregnate the sheet. On the other hand, if all short fibred cotton is used, the felt made on the cylinder machine will be too dense and will not stretch, nor can a mixture of all long wool and of long cotton fibres be felted 40 on a cylinder felting machine because it is too free to felt properly. If a mixture of all short cotton and all long wool fibres in which the cotton predominates be used, the sheet is too dense. The same is true of a mixture 45 of all short cotton and all short wool fibres in which the cotton predominates.

To the end, therefore, of providing a water-laid beaten felt which will avoid the disadvantages of existing felts, I have de- 50 vised my present invention. According to

it, I employ a mixture of textile rags containing a good percentage of relatively long fibres, which may be of animal, vegetable or mineral origin. This mixture is beaten out in accordance with usual practice in a beater 55 in the presence of water, and to it is added the shredded corium portions of certain animal skins, as for example, rabbit, deer, beaver or similar animals.

The action of the beater causes the 60 shredded corium, which is untanned, to yield an agglutinous substance which is probably the subcutaneous fat from the elastic fibres or dense connective tissue of the corium. This agglutinant is in the form of a fluid 65 gum, glue or gelatinous substance which adheres as long elastic tacky shreds to the long wool and cotton fibres of the fibrous base, and assists these fibres in their felting action by holding them together in interlaced or 70 matted condition, so that they will absorb sufficient water to felt satisfactorily on the cylinder felting machine and yet will be open and porous enough to hold the thermoplastic 75 binder, and at the same time will have sufficient capacity for stretch to enable the box toe blanks cut from the felt to be molded to proper shape when the shoe is lasted.

Broadly, therefore, my invention involves 80 the concept of adding to the fibrous mass the corium portions of the skins or pelts of certain animals which on treatment have the property of tending to cause the long fibres of the fibrous base to hold more water so that they can properly mat or felt on a cylinder 85 felting machine. More specifically, my invention involves the perception that the residual fluid gummy, gelatinous, or glutinous substance yielded by the corium under the action of the beater constitutes an effective agglutinant which will adhere to the long fibres of the fibrous base and will assist them in their felting action.

Because of its availability, I prefer to use 90 the shredded corium of untanned rabbit pelts or skins, although I may use other skins. Such a material is a standard by-product of the usual hat factory and is available in unlimited quantities.

Although proportions vary according to 100

the particular specifications of different box toe manufacturers and hence may widely differ in different cases, the following mix is given for purposes of illustration and as 5 representing a mix which will give a commercially satisfactory felt: To approximately 75% textile rags, that is mixtures of cotton and woolen rags so beaten out as to contain a good percentage of long fibres, I add approximately 25% shredded corium.

10 To this may be added, if desired a small percentage, approximately 1% of caustic soda, soda ash or similar material which will assist in bringing out the tackiness of the shredded corium.

15 In practicing my invention, the usual process is followed, that is to say, the fibrous base is beaten out in the presence of water in the beater until smooth but yet kept relatively 20 long as to length of fibre, whereupon the shredded corium, and if desired, the caustic soda or other colloidizing assistant is added to the mix and the beaten stock run on a cylinder felting machine. The stock is then 25 sheeted out and impregnated with a thermoplastic binder, as by dipping the sheet material into a fluid bath containing the binder.

30 I thus obtain a felt which is open and porous enough to hold the thermoplastic binder and yet has capacity for stretch sufficient to permit it to be molded over the last without danger of rupture or tear. The residual agglutinant yielded up by the shredded corium in the action of the beater adheres to 35 the long fibres of the fibrous base and assists them in their felting action, slowing down their water-absorbent tendency and so that the stock will felt satisfactorily on the cylinder felting machine.

40 While particularly useful as a box toe felt, my felt may, however, be used for the various other purposes to which the ordinary box toe felt is sometimes employed, as roofing or flooring felt.

45 Similarly, various modifications in fibre and fibre treatment may be made within the spirit and scope of my invention as defined by the appended claims.

50 What I therefore claim and desire to secure by Letters Patent is:

1. A porous water-laid felt having a preponderating proportion of long fibers bonded together with a smaller proportion of the 55 gelatinized corium portion of untanned animal skins.

2. A porous water-laid felt having a preponderating proportion of long fibers bonded together with a smaller proportion of the 60 gelatinized corium portion of untanned rabbit skins.

3. A strong porous water-laid felt comprising substantially 75% of fibrous material containing a substantial proportion of long 65 fibers, and substantially 25% of the gelatin-

ized corium portion of untanned animal skins bonding the fibers together.

4. A water-laid felt consisting of a beaten mixture of fibers and the shredded corium portions of untanned animal skins distributed therethrough and in relation therewith, the fibers being present in preponderating amount sufficient to cause the felt to be sufficiently open and porous to be readily saturated with a melted thermoplastic stiffening agent.

70 In testimony whereof I affix my signature.  
HENRY PHILIP SHOPNECK.

80

85

89

93

98

102

106

110

114

118

122